

# UNITED STATES PATENT OFFICE.

AUGUSTE J. ROSSI, OF NIAGARA FALLS, NEW YORK, ASSIGNOR TO THE TITANIUM ALLOY MANUFACTURING COMPANY, OF NEW YORK, N. Y., A CORPORATION OF MAINE.

## ALLOY OF THE PRECIOUS METALS AND METHOD OF INCREASING HARDNESS OF SUCH ALLOY.

1,023,334.

Specification of Letters Patent.

Patented Apr. 16, 1912.

No Drawing. Original application filed May 6, 1910, Serial No. 559,656. Divided and this application filed January 25, 1912. Serial No. 673,359.

*To all whom it may concern:*

Be it known that I, AUGUSTE J. ROSSI, a citizen of the United States, and a resident of Niagara Falls, in the county of Niagara and State of New York, have invented certain new and useful Improvements in Alloys of the Precious Metals and Methods of Increasing Hardness of Such Alloys, of which the following is a specification.

10 My present application for patent is a division of my previous application Ser. No. 559,656, filed May 6, 1910.

15 My present invention relates to the hardening of such alloys including particularly such as used in coinage, jewelry and the like, and has for its object the imparting to such alloys so employed and containing present conventional proportions of copper, such novel increased hardness as will enable 20 them to better resist frictional wear to which they may be subjected.

25 As well understood, the precious metals, *i. e.* gold and silver, are inherently so soft as to lose important proportions of their weight by the wear to which subjected when employed in coins, jewelry, or the like. It has therefore from time immemorial been the practice to alloy for such uses one of the 30 said precious metals with various proportions of a harder metal, as copper, the gold and silver coinage of most countries being correspondingly debased by intentional additions of copper varying from 9 to 10% or thereabout, and the said alloys intended 35 for commercial uses and commonly known as "sterling" gold, or "sterling" silver containing as high as 25% of copper. Notwithstanding these admixtures of the baser metal, the resulting coinage, money, bars, 40 jewelry, etc. are still nevertheless subject to important undesired losses from friction and wear in use, and the object of my present invention is to provide means for preventing such losses and the production 45 of articles comparatively not subject thereto.

45 I have discovered that if to either of the said "precious metals," while molten, there be added the present usual conventional proportions of a copper previously purified by 50 titanium, as per Letters Patent No. 905,232, granted to me December 1, 1908, or alloyed with titanium as per Letters Patent No.

935,863, granted to me October 5, 1909, or there be added to such precious metal, when molten together with the desired per cent. of 55 previously unpurified or unalloyed copper, a small amount of titanium, or of my said alloy of copper with titanium, the final resulting alloy of said precious metal with copper will be so hardened as to substantially resist, without loss of weight, substantially all wear incident to ordinary usage.

55 My invention may be practiced as follows: The copper intended for use in hardening the precious metal whether gold or silver as aforesaid is first melted and to the molten bath thereof is added and melted therewith some of my alloy or compound of copper and titanium for which Reissued 70 Letters Patent No. 12,764 were on March 17, 1908, granted to me, the amount of said alloy so added being preferably proportioned to insure in the bath the presence of 75 sufficient metallic titanium to combine with undesired elements and compounds present and leave a final copper product containing substantially no titanium, or, if desired, not to exceed 1% of titanium as per my said Letters Patent No. 905,232. The resulting 80 purified copper product is then added to a bath of the molten precious metal, *i. e.* gold or silver as the case may be, and in such proportion as to secure in the final product or alloy the desired proportion of copper. 85 The said resulting final product, being an alloy of gold or silver with copper, should contain not to exceed traces of titanium and will therefore be of substantially the same purity as formerly required for coinage and 90 commercial uses aforesaid, but its resistance to abrasion will be found much greater than that of a corresponding alloy to which, or its constituents, the titanium has not been 95 added.

95 It will be obvious that substantially the same results may be attained by adding to a bath of either molten gold or molten silver a certain amount of copper not previously treated with titanium as aforesaid and then 100 also adding sufficient of my said alloy of copper and titanium, containing a sufficient percentage of titanium, to impart to the bath as a whole enough metallic titanium to com-

bine with all undesired elements and compounds present in said bath and leave in the final product thereof substantially no titanium.

- 5 I am satisfied that notwithstanding usually accepted comparative purity of the precious metals gold and silver, these nevertheless do contain in their usual commercial condition as raw materials more or 10 less of undesired impurities and compounds, which tend to impart to the mass undesirable susceptibility to abrasion and wear. Such impurities are, I believe, beneficially effected or removed through the action of 15 the titanium when added as last above mentioned, and I therefore suggest that whenever analysis or other test discloses such impurities, care be taken to proportion the titanium added so as to insure its action 20 thereon as well as on undesired elements, compounds and impurities imported into the bath by the copper thereto added.

It will be understood that where the presence of some titanium *per se* may be unobjectionable, as for uses other than coinage, the titanium introduced may be so proportioned as to leave in the final product a decided percentage of titanium, say up to 1%, or thereabout, whereby in some instances 30 greater resistance to abrasion may be imparted than when the titanium has been proportioned to leave only traces, or substantially no titanium in the final product.

It will be understood that my invention, as herein claimed, is limited to methods of 35 treatment of gold, or its alloys, in which the titanium employed is of such proportion as to leave in the final resulting product more than traces of titanium.

What I claim as new and desire to secure 40 by Letters Patent is the following, viz:—

1. The metallurgical method which comprises bringing together in molten state gold, a harder metal, and titanium.
2. The metallurgical method which comprises bringing together in molten state gold, copper and titanium.
3. The method of producing an alloy of gold with a harder metal which comprises bringing together in molten state gold and 50 an alloy of said harder metal with titanium.
4. The method of producing an alloy of gold with a harder metal which comprises bringing together in molten state gold and an alloy of copper with titanium.

5. As a new article, a metallic substance composed principally of gold, a harder metal therewith alloyed, and some titanium.

6. As a new article, a metallic substance composed principally of gold, copper there- 60 with alloyed, and some titanium.

AUGUSTE J. ROSSI.

Witnesses:

WALTER D. EDMONDS,  
PHILIP C. PECK.